

2,745,739

## STEEL GLASS SEALS AND STEEL THEREFOR

Freeman J. Phillips, Pittsburgh, and Charles O. Tarr, McKeesport, Pa., assignors to United States Steel Corporation, a corporation of New Jersey

No Drawing. Application October 22, 1952,  
Serial No. 316,326

6 Claims. (Cl. 75—128)

This invention relates to steel glass seals wherein the 15 steel is a chromium stainless steel containing 9.5 to 13.5% chromium and more particularly is a stainless steel of this type that is ferritic at all temperatures up to 1200° C. and also has a coefficient of expansion closely approximating that of expansion of glass particularly on 20 cooling through the range of 530 to 30° C.

In sealing glass to metal, the temperature of the glass is raised to fusion point of glass, i. e., about 1200° C. to effect the seal. If the seal is to remain intact without shattering or placing undue strain on the glass, the coefficients of expansion of the glass and the metal must be closely matched on cooling, particularly throughout the range of temperature 530° to 30° C. Moreover, for many purposes such as cones for television tubes and the like, it is necessary to form the metal articles in a spinning operation. Due to their ready formability, chromium stainless steels of the 28-30% straight chromium type and modified 17% grades of such steel have heretofore been used for such purpose. While such steels are quite satisfactory, they are quite expensive and it is therefore desirable to use cheaper grades of steel. We discovered that stainless steel containing 9.5 to 13.5% chromium can be used for such purpose if modified as hereinafter set forth.

It is accordingly an object of the present invention to 40 provide chromium stainless steels suitable for forming by spinning and for sealing to glass containing less chromium than steels heretofore usable.

It is a further object of the present invention to render stainless steels containing 9.5 to 13.5% chromium suitable for sealing to glass.

The foregoing and further objects of this invention will be apparent from the following invention which is directed generally to chromium stainless steels containing 9.5 to 13.5% chromium.

Steels of this type are readily formable by spinning and are sufficiently oxidation resistant to make them desirable for use in applications requiring that glass be sealed thereto. Moreover, they are considerably cheaper than steels heretofore used. They, however, form austenite upon heating to high temperatures which partially transforms to martensite upon cooling. The accompanying changes in volume, causing an unfavorable coefficient of expansion render them unsuitable for sealing to glass. Also, to be suitable for sealing to glass the steel should have a coefficient of expansion over the temperature range of 530° to 30° C. of less than  $12.5 \times 10^{-6}$  in./in./° C., preferably being within the range of about 11.5 to  $12.5 \times 10^{-6}$  in./in./° C.

We have discovered that chromium steels within the range of 9.5 to 12.5% chromium containing less than .10% carbon are generally suitable if they contain at least .50% titanium along with .25 to about 1.00% molybdenum, aluminum within the range of .02 to .30%, silicon .10 to 1.00%, manganese .10 to .75% and less than .50% nickel. While the upper limit of titanium is not critical with respect to the purposes of the invention, it is gener-

ally maintained below about 1% since larger amounts cause objectionable stringers. Phosphorus and sulphur should be maintained as low as possible. Small quantities of boron, vanadium and tungsten are not desirable, but may be tolerated. The balance of the alloy is substantially iron.

Steels within the foregoing ranges will generally be ferritic and have a suitable coefficient of expansion. To ensure the steel being completely ferritic, the amounts of the desired elements present should be regulated in accordance with the formula:

$$\% \text{Cr} + \% \text{Si}/2 + 30 \times \% \text{Ti} + 10 \times \% \text{Al} + 2.4 \times \% \text{Mo} - 4.27 (\% \text{Ni} + \% \text{Mn}/2 \times \% \text{C}) - 19.56 = \text{a sum greater than unity}$$

Thus if the result is positive, the steel will be completely ferritic whereas if the result is negative, both ferrite and martensite may be present after quenching from 1200° C.

The following table lists the analyses of a number of steels embodying our invention:

Table I

|      | C    | Mn  | P    | S    | Si  | Ni  | Cr    | Ti  | Mo  | Al  |
|------|------|-----|------|------|-----|-----|-------|-----|-----|-----|
| 25 A | .060 | .54 | .011 | .015 | .26 | .33 | 9.85  | .66 | .53 | .16 |
| B    | .058 | .59 | .012 | .017 | .34 | .34 | 13.30 | .58 | .53 | .15 |
| C    | .064 | .55 | .008 | .010 | .19 | .39 | 10.85 | .55 | .90 | .11 |
| D    | .028 | .64 | .009 | .012 | .16 | .39 | 10.72 | .54 | .84 | .12 |

All of these steels were completely ferritic after heating to 1200° C. and quenching and the coefficients of expansion on cooling from 530° to 30° C. were within the range of  $11.5$  to  $12.5 \times 10^{-6}$  in./in./° C. Steel A, for example, had a coefficient of expansion of 12.04, steel C, 12.0 and steel D,  $11.9 \times 10^{-6}$  in./in./° C.

As is shown by the following Table II, steels outside the above ranges are unsatisfactory since they were observed to have both the ferrite and the martensite phases after heating to 1200° C. and quenching:

Table II

|   | C    | Mn  | P    | S    | Si  | Ni  | Cr   | Ti  | Mo  | Al   |
|---|------|-----|------|------|-----|-----|------|-----|-----|------|
| E | .066 | .54 | .011 | .017 | .30 | .18 | 9.78 | .21 | .52 | .015 |
| F | .068 | .52 | .012 | .017 | .27 | .18 | 9.74 | .21 | .52 | .213 |
| G | .04  | .53 | .010 | .011 | .16 | .40 | 9.11 | .50 | .92 | .09  |

While we have shown and described several specific embodiments of our invention, it will be understood that these embodiments are merely for the purpose of illustration and description and that various other forms may be devised within the scope of our invention, as defined in the appended claims.

We claim:

1. A stainless steel characterized by being ferritic completely after heating to 1200° C. and quenching, and having a coefficient of expansion of less than  $12.5 \times 10^{-6}$  in./in./° C. throughout the temperature range of 530° to 30° C. containing 9.5 to 13.5% chromium, less than .10% carbon, at least .50% titanium, .25 to 1.00% molybdenum, .02 to .30% aluminum, .10 to 1.00% silicon, .10 to .75% manganese and less than .50% nickel, said chromium, carbon, titanium, molybdenum, aluminum, silicon, manganese and nickel being restricted to amounts consistent with the formula

$$\% \text{Cr} + \% \text{Si}/2 + 30 \times \% \text{Ti} + 10 \times \% \text{Al} + 2.4 \times \% \text{Mo} - 4.27 (\% \text{Ni} + \% \text{Mn}/2 \times \% \text{C}) - 19.56 = \text{a sum greater than unity}$$

2. A stainless steel characterized by being ferritic completely after heating to 1200° C. and quenching, and having a coefficient of expansion of less than  $12.5 \times 10^{-6}$  in./in./° C. throughout the temperature

range of 530° to 30° C. containing 9.5 to 13.5% chromium, less than .10% carbon, at least .50% titanium, .25 to 1.00% molybdenum, .02 to .30% aluminum, .10 to 1.00% silicon, .10 to .75% manganese and less than .50% nickel with the balance substantially iron and residual impurities, said chromium, carbon, titanium, molybdenum, aluminum, silicon, manganese and nickel being restricted to amounts consistent with the formula



3. A method of forming stainless steel suitable for forming by a spinning operation and sealing to glass, said steel containing 9.5 to 13.5% chromium, less than .10% carbon, at least .50% titanium, .25 to 1.00% molybdenum, .02 to .30% aluminum, .10 to 1.00% silicon, .10 to .75% manganese and less than .50% nickel, comprising melting the steel and controlling the amounts of the foregoing elements therein in accordance with the formula



said steel being characterized by being completely ferritic after heating to 1200° C. and quenching and by having a coefficient of expansion of less than  $12.5 \times 10^{-6}$  in./in./° C. throughout the temperature range of 530° to 30° C.

4. A method of forming stainless steel suitable for forming by a spinning operation and sealing to glass, said steel containing 9.5 to 13.5% chromium, less than .10% carbon, at least .50% titanium, .25 to 1.00% molybdenum, .02 to .30% aluminum, .10 to 1.00% silicon, .10 to .75% manganese and less than .50% nickel, comprising melting the steel and controlling the amounts of the foregoing elements therein in accordance with the formula



with the balance substantially iron and residual impurities, said steel being characterized by being completely ferritic after heating to 1200° C. and quenching and by having a coefficient of expansion of less than  $12.5 \times 10^{-6}$  in./in./° C. throughout the temperature range of 530° to 30° C.

5. A glass to steel seal wherein the glass is heated to its fusion point while in direct contact with the steel, the

steel being a ferritic stainless steel containing 9.5 to 13.5% chromium, less than .10% carbon, at least .50% titanium, .25 to 1.00% molybdenum, .02 to .30% aluminum, .10 to 1.00% silicon, .10 to .75% manganese and less than .50% nickel, said chromium, carbon, titanium, molybdenum, aluminum, silicon, manganese and nickel being restricted to amounts consistent with the formula



said steel being characterized by being completely ferritic after heating to 1200° C. and quenching and by having a coefficient of expansion of less than  $12.5 \times 10^{-6}$  in./in./° C. throughout the temperature range of 530° to 30° C.

6. A glass to steel seal wherein the glass is heated to its fusion point while in direct contact with the steel, the steel being a ferritic stainless steel containing 9.5 to 13.5 chromium, less than .10% carbon, at least .50% titanium, .25 to 1.00% molybdenum, .02 to .30% aluminum, .10 to 1.00% silicon, .10 to .75% manganese and less than .50% nickel with the balance substantially iron and residual impurities, said chromium, carbon, titanium, molybdenum, aluminum, silicon, manganese and nickel being restricted to amounts consistent with the formula



said steel being characterized by being completely ferritic after heating to 1200° C. and quenching and by having a coefficient of expansion of less than  $12.5 \times 10^{-6}$  in./in./° C. throughout the temperature range of 530° to 30° C.

#### References Cited in the file of this patent

#### UNITED STATES PATENTS

- |           |        |               |
|-----------|--------|---------------|
| 1,947,417 | Holst  | Feb. 13, 1934 |
| 2,024,561 | Becket | Dec. 17, 1935 |
| 2,670,572 | Smith  | Mar. 2, 1954  |

#### FOREIGN PATENTS

- |         |         |              |
|---------|---------|--------------|
| 730,161 | Germany | Jan. 7, 1943 |
|---------|---------|--------------|

#### OTHER REFERENCES

- 50 Metal Progress, vol. 52, July to December publications, pages 94 to 96, and 102. Published by the American Society for Metals, Cleveland, Ohio.